

## UNITED STATES PATENT OFFICE

2,515,122

## PROCESS FOR PREVENTING STAINS IN PHOTOGRAPHIC COLOR MATERIAL BY THE USE OF A FIXING BATH CONSISTING OF WATER, AN ALKALI SULFITE, AND A FIXING AGENT

Harold C. Harsh and James E. Bates, Binghamton, N. Y., assignors to General Aniline & Film Corporation, New York, N. Y., a corporation of Delaware

No Drawing. Application December 3, 1945,  
Serial No. 632,592

9 Claims. (Cl. 95—88)

1

This invention relates to photographic anti-stain baths, to anti-stain baths employed in multi-color photography, and especially to non-staining baths for the fixing of multi-color photographic material following the bleaching treatment.

It is known that in the processing of multi-color reversible film and multi-color reversible white opaque, the exposed film or exposed white opaque, is first developed with a normal black and white developer to produce a negative image. After development, the black and white negative material, without being fixed, is exposed to general illumination, followed by a second development with a color-forming developer. During the first and second development the silver-halides in all the layers are reduced to metallic silver. After the second development, the material is cleared in running water, hardened in an aqueous solution consisting of either chrome or potassium alum, and then washed in running water. After the latter treatment, the silver present in all the layers formed during the first and second development is converted into a salt by any of the known silver-salt formers, commonly known as bleaching baths, and the silver-salt thus formed is then removed by dissolving it in a silver-salt solvent such as, for example, hypo. The material is then washed for a long period of time and then dried.

Prior to the washing operation it is essential that the residual second or color developer and bleach solutions be removed, otherwise stains will be formed during the washing and drying operations, which are particularly noticeable in the white area. In order to prevent this staining, an extended final washing time in running water of from fifteen minutes to two hours, has been proposed. Even if this proposal be adopted, stains are nevertheless formed during the long washing operation, which makes it imperative to keep the washing time as short as possible. However, if washing times are reduced so that the staining is kept to a minimum, the chemicals will not be eliminated from the emulsion layers and stains will form during drying. It is believed that the staining results from the oxidation of traces of the color developer retained in the layers of the material following color-forming development, when then react with the unused color-former.

2

An object of the present invention is to permit normal washing time of color developed multi-color photographic material while preventing the formation of stain.

5 Another object is to permit a shorter washing time than is normally required while preventing staining during both the final washing and drying operations.

A further object of the invention is a fixing 10 bath which clears undesirable matter from a multi-color photographic material in a short time while avoiding staining.

Other objects and features of the invention will 15 become more apparent as the description proceeds.

We have found that the above objects are accomplished by employing, as a fixing bath, an aqueous solution containing hypo such as ammonium thiosulfate or sodium thiosulfate, and a 20 water soluble alkali sulfite such as ammonium, potassium or sodium sulfite, bisulfite, and meta bisulfite. This discovery makes it possible to considerably reduce the final washing time. The concentration of hypo may vary from 100 grams to 25 300 grams per liter of water. The concentration of the water-soluble alkali sulfite may vary from 1 gram to as high as 20 grams per liter. The concentration of the hypo and the alkali sulfite should be so adjusted that the pH of the resulting solution is not lower than a pH of 6.0. Amounts of alkali sulfite higher than 20 grams per liter give little improvement in stain prevention from a practical standpoint and, accordingly, concentrations ranging from between 1 to 15 grams 35 per liter are most desirable.

The photographic multi-layer materials, which 40 may be processed with the anti-stain bath of the present invention, are color reversible film, color negative film, color reversible white opaque, and color paper irrespective of whether the dyestuff images are produced with the color-formers incorporated in the emulsion or by a selective second exposure and color development wherein the color-formers are added to the developing solution. The color reversible film consists of an integral tripack emulsion coated on the usual clear cellulose acetate or nitrate film base. Each of the emulsions are sensitized to one of the primary colors of light, namely, blue, green, and red. 45 The top layer is blue sensitive. A filter layer,

## 3

yellow in color and blue absorbing, lies under the top layer. Below this filter layer, lies a green sensitive emulsion layer, and below this is a red sensitive emulsion layer. Each of the three silver-halide emulsion layers contain dye-forming compounds which unite during the development of silver image in an aromatic amine developing agent to form a dye with the oxidation product of the developing agent, or may be free from color-formers in which case the film is processed with the color-formers in the color developers by the selective second exposure and color development method as described in United States Patents 1,897,866; 1,900,870; 1,928,709 and 1,980,941. The color negative film is made up in the same manner as the color reversible film, with the exception that it may contain a layer of clear gelatin between the red sensitive layer and the green sensitive layer. The color reversible white opaque material is prepared in the same manner as color reversible film and the color negative film, with the exception that the base consists of an opaque white film. The color paper is also constructed in the same manner as the color reversible film and the color negative film, with the exception that the emulsion is coated on a baryta coated paper base.

As silver is formed during development, it must be removed after color development by treatment in a bleach, followed by treatment in a bath of sodium thiosulfate according to usual practice. A yellow dye is formed in the blue sensitive emulsion; a magenta dye is formed in the green sensitive emulsion; and a cyan dye is formed in the red sensitive emulsion. Combinations of these three printing primaries will produce all of the other colors in the finished film or print. Suitable methods for the preparation of photographic multilayer materials have been described in the literature relating to color photography, and are, therefore, not described here.

The following examples describe in detail methods for accomplishing the above objects, but it is to be understood that they are inserted merely for the purpose of illustration and are not to be construed as limiting the scope of the invention.

*Example I*

A 4" x 5" full color transparency sheet of color film was printed by contact on two 4" x 5" sheets of color reversible white opaque film.

The two sheets of 4" x 5" color reversible white opaque film were first developed for twelve minutes at 68° F. in a developer of the following composition:

|                                    |          |    |
|------------------------------------|----------|----|
| p-Monomethylamine-m-phenol sulfate | grams... | 3  |
| Sodium sulfite                     | do...    | 50 |
| Hydroquinone                       | do...    | 6  |
| Sodium carbonate (monohydrate)     | do...    | 40 |
| Sodium thiocyanate                 | do...    | 2  |
| Potassium bromide                  | do...    | 2  |
| Water to make up                   | liter... | 1  |

Short stopped for 3 minutes at 68° F., in a 5% aqueous solution of sodium bisulfite.

Washed for 2 minutes in running water at 68° F.

Color developed for 15 minutes at 68° F., in a developer of the following composition:

|                           |          |    |
|---------------------------|----------|----|
| p-Aminodiethylaniline HCl | grams... | 4  |
| Sodium sulfite            | do...    | 5  |
| Hydroxylamine HCl         | do...    | 2  |
| Sodium carbonate          | do...    | 40 |
| Potassium bromide         | do...    | 1  |
| Water to make up          | liter... | 1  |

## 4

Rinsed for 4 minutes in running water at 68° F. Hardened for 5 minutes in a 3% aqueous solution of potassium chrome alum.

Washed for 5 minutes in running water at 68° F. The washed material was then treated with a bleach bath of the following composition:

|                                       |          |     |
|---------------------------------------|----------|-----|
| Di-potassium mono-sodium ferricyanide | grams... | 100 |
| Potassium bromide                     | do...    | 15  |
| Disodium phosphate                    | do...    | 40  |
| Sodium bisulfite                      | do...    | 25  |
| Formalin (40%)                        | cc...    | 20  |
| Water to make up                      | liter... | 1   |

Washed for 5 minutes at 68° F.

The first washed film was fixed in solution No. 1 and the second washed film was fixed in solution No. 2 of the following compositions:

|                    | No. 1     | No. 2 |
|--------------------|-----------|-------|
| Sodium thiosulfate | grams...  | 200   |
| Sodium sulfite     | do...     | 5     |
| Water to make up   | liters... | 1     |

The two fixed film sheets were then washed in water from 10-20 minutes. At this point the films appeared identical. After normal drying, the film fixed in solution No. 1 showed objectionable stains, while the film fixed in solution No. 2 containing sodium sulfite was clear and unstained.

When the drying was carried out under conditions of high humidity so that the drying time was extended for several hours, the film fixed in solution No. 1 showed even greater highlight stains, while the film fixed in solution 2 containing sodium sulfite did not change.

*Example II*

Example I was repeated with the exception that the colored photographic multilayer material employed was color paper and the fixing solution No. 2 contained 3 grams of sodium bisulfite instead of 5 grams of sodium sulfite. The color print fixed in solution No. 1 showed objectionable stains after washing and drying, while the print fixed in solution No. 2 containing sodium bisulfite after washing and drying was clear and unstained.

*Example III*

Example I was repeated with the exception that the fixing solution No. 2 contained 3 grams of sodium metabisulfite instead of sodium sulfite. After fixing, washing and drying, the color print fixed in solution No. 1 showed objectionable stains, while the print fixed in solution No. 2 containing sodium metabisulfite was clear and unstained.

From the above examples, it is manifest that multilayer photographic material fixed in an ordinary hypo solution shows marked staining after washing and drying of said material. This staining occurs especially under slow drying conditions and is probably due to the coupling of the slow oxidation product of the color developer with a residual color coupler present in one or more layers.

It will be understood that where in the claims appended hereto the term "hypo" is used, that such is intended to include ammonium thiosulfate.

This application is a continuation-in-part of our co-pending application Serial No. 627,533, filed on November 8, 1945, now Patent No. 2,475,134, July 5, 1949.

The above specific examples are to be regarded as merely illustrative of the invention, and not in

any sense restrictive. It will be obvious to anyone skilled in the art that many modifications such as substituting equivalent material and varying the proportions of materials used are within the spirit and scope of the invention as defined in the appended claims.

We claim:

1. In the process of color photography, the method of preventing stains on color images selected from the class consisting of indophenol and azomethine dyes produced in multilayer color film by color forming development which comprises fixing said film after exposure, color development, and bleaching with an aqueous solution consisting of water, an alkali sulfite, and a fixing agent of the group consisting of ammonium thiosulfate and sodium thiosulfate, and thereafter washing and drying the fixed film.

2. In the process of color photography, the method of preventing stains on color images selected from the class consisting of indophenol and azomethine dyes produced in multilayer color film by color forming development which comprises fixing said film after exposure, color development, and bleaching with an aqueous solution consisting of water, sodium sulfite, and a fixing agent of the group consisting of ammonium thiosulfate and sodium thiosulfate, and thereafter washing and drying the fixed film.

3. In the process of color photography, the method of preventing stains on color images selected from the class consisting of indophenol and azomethine dyes produced in multilayer color film by color forming development which comprises fixing said film after exposure, color development, and bleaching with an aqueous solution consisting of water, sodium bisulfite, and a fixing agent of the group consisting of ammonium thiosulfate and sodium thiosulfate, and thereafter washing and drying the fixed film.

4. In the process of color photography, the method of preventing stains on color images selected from the class consisting of indophenol and azomethine dyes produced in multilayer color film by color forming development which comprises fixing said film after exposure, color development, and bleaching with an aqueous solution consisting of water, sodium metabisulfite, and a fixing agent of the group consisting of ammonium thiosulfate and sodium thiosulfate, and thereafter washing and drying the fixed film.

5. The method according to claim 1, wherein the concentration of the said alkali sulfite ranges from 1 to 20 grams per liter.

6. In a process of producing color photographic images selected from the class consisting of indophenol and azomethine dyes in a multilayer color film by exposing the film, color developing the same, bleaching, and washing, the improvement which comprises avoiding the formation of stain, after the bleaching and washing operation, by fixing the said film with an aqueous solution consisting of water, an alkali sulfite, and a fixing

agent of the group consisting of ammonium thiosulfate and sodium thiosulfate, and thereafter washing and drying the fixed film.

7. In a process of producing color photographic images selected from the class consisting of indophenol and azomethine dyes in a multilayer color film by exposing the film, color developing the same, bleaching, and washing, the improvement which comprises avoiding the formation of stain, after the bleaching and washing operation, by fixing the said film with an aqueous solution consisting of water, sodium sulfite, and a fixing agent of the group consisting of ammonium thiosulfate and sodium thiosulfate, and thereafter washing and drying the fixed film.

8. In a process of producing color photographic images selected from the class consisting of indophenol and azomethine dyes in a multilayer color film by exposing the film, color developing the same, bleaching, and washing, the improvement which comprises avoiding the formation of stain, after the bleaching and washing operation, by fixing the said film with an aqueous solution consisting of water, sodium bisulfite, and a fixing agent of the group consisting of ammonium thiosulfate and sodium thiosulfate, and thereafter washing and drying the fixed film.

9. In a process of producing color photographic images selected from the class consisting of indophenol and azomethine dyes in a multilayer color film by exposing the film, color developing the same, bleaching, and washing, the improvement which comprises avoiding the formation of stain, after the bleaching and washing operation, by fixing the said film with an aqueous solution consisting of water, sodium metabisulfite, and a fixing agent of the group consisting of ammonium thiosulfate and sodium thiosulfate, and thereafter washing and drying the fixed film.

40 HAROLD C. HARSH.  
JAMES E. BATES.

#### REFERENCES CITED

The following references are of record in the 45 file of this patent:

#### UNITED STATES PATENTS

|    | Number    | Name            | Date           |
|----|-----------|-----------------|----------------|
| 50 | 1,521,840 | Sheppard        | Jan. 6, 1925   |
|    | 1,544,936 | Punnett         | July 7, 1925   |
|    | 1,753,059 | Murray          | Apr. 1, 1930   |
|    | 1,976,301 | Seymour et al.  | Oct. 9, 1934   |
|    | 2,059,884 | Mannes          | Nov. 3, 1936   |
|    | 2,063,297 | Crabtree et al. | Dec. 8, 1936   |
| 55 | 2,203,903 | Ham             | June 11, 1940  |
|    | 2,323,481 | McQueen         | July 6, 1943   |
|    | 2,384,658 | Vittum          | Sept. 11, 1945 |
|    | 2,414,491 | Tulagin         | Jan. 21, 1947  |

#### OTHER REFERENCES

60 Clerc, "Photography Theory and Practice," 2d edition, 1937, published by Sir Isaac Pitman & Sons Ltd., pages 236 and 237 cited.